

# ALIEN PROPERTY CUSTODIAN

2,324,630

## PATENTING STEEL

Elmer E. Legge, West Hartford, Conn.

No Drawing. Application May 4, 1942,  
Serial No. 441,678

### 3 Claims. (Cl. 148—21)

This invention is concerned with patenting steel by means of a liquid patenting quench bath, the object being to produce a more uniformly patented structure than has heretofore been possible.

Conventionally, the steel, usually in the form of rod or wire, is continuously moved through an austenitizing heating zone, provided by either a continuous furnace or a high temperature lead bath, and is then continuously moved through the liquid patenting quench bath, which may be either a molten salt or lead bath. The steel must enter the patenting quench bath while it is still austenitic from its passage through the austenitizing heating zone, which means that when the steel enters it is at a much higher temperature than that of the patenting quench bath. Furthermore, the steel necessarily enters the patenting quench bath continuously at the same location, and travels therethrough in the same path during its patenting, thus producing a high temperature zone in the patenting quench bath surrounding the steel's entering location and which decreases gradually in temperature to indeterminable distances therebeyond, where it becomes merged with the patenting quench bath.

As a result of the above practice, the steel's austenite transforms, as the steel passes through the patenting quench bath, at widely varying temperatures imparting a mixed structure to the steel ranging from very coarse pearlite to relatively fine pearlite, or sorbite, it being understood that patenting is carried out in the temperature range where austenite very rapidly transforms to pearlite, namely, within the temperature range of from 800° to 1350° F. It is most desirable to produce a uniform structure consisting throughout of the austenite transformation product inherent to the specific patenting temperature at which the patenting quench bath is maintained, it being otherwise impossible to accurately predict the properties of the patented steel.

According to the present invention, the foregoing practice is improved by continuously moving the austenitized steel leaving the austenitizing heating zone and prior to its entering the patenting quench bath, through a liquid pre-quench bath having a substantially lower temperature than the patenting quench bath with suitable length reducing the temperature of the steel at least approximately to that of the patenting quench in a time period too short to permit more than minor amounts of the steel's austenite to transform, whereby the steel enters

the patenting quench in at least a mainly austenitic condition at a temperature not substantially higher than that of this quench and thus avoids the formation therein of a high temperature zone.

This liquid prequench bath may consist of any suitable quenching liquid, it functioning to rapidly abstract the heat imparted to the steel as it moved through the austenitizing heating zone, 10 preferably without permitting any austenite transformation, the steel then entering the patenting quench bath at almost the same temperature of this bath, or even at a slightly lower temperature. The formation of a widely varying 15 temperature zone in the prequench bath is immaterial since there is little or no austenite transformation effected therein, it functioning merely to abstract heat from the steel. A high temperature zone cannot occur in the patenting quench bath. Should a low temperature zone occur in the entering end of the patenting quench bath, any austenite transformation occurring in this zone will produce a structure that will automatically be tempered as the remainder of the austenite goes to the patented structure, and will result in a tempered product having substantially 20 the same physical properties as this patented structure.

The temperature of the prequenching bath 30 should preferably range from 350° to 700° F., while patenting temperatures are herein considered as ranging from 800° to 1350° F., this last range applying to the patenting quench bath. This patenting range is advanced since it represents the temperature range where austenite very 35 rapidly transforms to pearlite, and, therefore, involves the problem solved by this invention; very fine pearlite, or sorbite, being produced at the lower limits of the range, and very coarse 40 pearlite being produced at the upper limits of the range. The exact temperature of the prequenching bath will depend on its length and the moving speed of the steel, it being preferable to co-relate these factors so that the steel enters the patenting quench bath at substantially the same temperature as that of the latter, but any variation in the temperature of the steel entering the quench bath should be lower than, rather than higher than, the patenting quench bath temperature.

It is obvious that this invention is particularly applicable to the patenting of wire and rod, and that it permits providing these products with a uniformly patented structure throughout. It is to be noted that the problem, solved by this in-

vention, is not present when austenitized steel is quenched at temperatures below those causing the rapid transformation of austenite to pearlite, because, in such instance, there is sufficient time for the steel to acquire the temperature of the quenching bath before its austenite starts to transform. In such instances, the practice of prequenching is for other purposes not connected with the problem solved by the present invention, this accounting for the reason that the prequenching disclosed herein has been unobvious to those skilled in the art in connection with patenting.

I claim:

1. In the art of patenting steel by continuously moving it successively through an austenitizing heating zone and a liquid patenting quench maintained at a temperature within the range causing rapid transformation of austenite to pearlite, the improvement comprising continuously moving the austenitized steel leaving said zone and prior to its entering said quench, through a liquid prequench having a temperature and length reducing the temperature of the steel at least approximately to that of the patenting quench in a time period too short to permit more than minor amounts of the steel's austenite to transform, whereby the steel enters the patenting quench at a temperature not substantially higher than that of this quench and

avoids the formation therein of a higher temperature zone.

2. A method of patenting steel, comprising continuously moving the steel through a heating zone rendering the steel austenitic, moving the austenitic steel through a liquid prequench maintained at a temperature within the range of from 350° to 700° F. for a time sufficient to reduce the steel's temperature substantially to within the range of from 800° to 1350° F., and, prior to more than minor amounts of the steel's austenite transforming, moving the steel through a liquid patenting quench maintained throughout at a temperature within the range of from 800° to 1350° F.
3. A method of patenting steel, comprising continuously moving the steel through a heating zone rendering the steel austenitic, moving the austenitic steel through a liquid prequench maintained at a temperature within the range of from 350° to 700° F. for a time sufficient to reduce the steel's temperature substantially to within the range of from 800° to 1350° F., and prior to more than minor amounts of the steel's austenite transforming, moving the steel through a liquid patenting quench maintained throughout at a temperature within the range of from 800° to 1350° F., said prequench time being sufficient to reduce the steel's temperature at least to that of the patenting quench.

ELMER E. LEGGE.

CERTIFICATE OF CORRECTION.

Patent No. 2,324,630.

July 20, 1943.

ELMER E. LEGGE.

It is hereby certified that error appears in the above numbered patent requiring correction as follows: Page 1 of the printed specification, near the top thereof, strike out the words "ALIEN PROPERTY CUSTODIAN" and insert instead --UNITED STATES PATENT OFFICE--; and that the said Letters Patent should be read with this correction therein.

Signed and sealed this 21st day of September, A. D. 1943.

(Seal)

Henry Van Arsdale,  
Acting Commissioner of Patents.

vention, is not present when austenitized steel is quenched at temperatures below those causing the rapid transformation of austenite to pearlite, because, in such instance, there is sufficient time for the steel to acquire the temperature of the quenching bath before its austenite starts to transform. In such instances, the practice of prequenching is for other purposes not connected with the problem solved by the present invention, this accounting for the reason that the prequenching disclosed herein has been unobvious to those skilled in the art in connection with patenting.

I claim:

1. In the art of patenting steel by continuously moving it successively through an austenitizing heating zone and a liquid patenting quench maintained at a temperature within the range causing rapid transformation of austenite to pearlite, the improvement comprising continuously moving the austenitized steel leaving said zone and prior to its entering said quench, through a liquid prequench having a temperature and length reducing the temperature of the steel at least approximately to that of the patenting quench in a time period too short to permit more than minor amounts of the steel's austenite to transform, whereby the steel enters the patenting quench at a temperature not substantially higher than that of this quench and

avoids the formation therein of a higher temperature zone.

2. A method of patenting steel, comprising continuously moving the steel through a heating zone rendering the steel austenitic, moving the austenitic steel through a liquid prequench maintained at a temperature within the range of from 350° to 700° F. for a time sufficient to reduce the steel's temperature substantially to within the range of from 800° to 1350° F., and, prior to more than minor amounts of the steel's austenite transforming, moving the steel through a liquid patenting quench maintained throughout at a temperature within the range of from 800° to 1350° F.
3. A method of patenting steel, comprising continuously moving the steel through a heating zone rendering the steel austenitic, moving the austenitic steel through a liquid prequench maintained at a temperature within the range of from 350° to 700° F. for a time sufficient to reduce the steel's temperature substantially to within the range of from 800° to 1350° F., and prior to more than minor amounts of the steel's austenite transforming, moving the steel through a liquid patenting quench maintained throughout at a temperature within the range of from 800° to 1350° F., said prequench time being sufficient to reduce the steel's temperature at least to that of the patenting quench.

ELMER E. LEGGE.

CERTIFICATE OF CORRECTION.

Patent No. 2,324,630.

July 20, 1943.

ELMER E. LEGGE.

It is hereby certified that error appears in the above numbered patent requiring correction as follows: Page 1 of the printed specification, near the top thereof, strike out the words "ALIEN PROPERTY CUSTODIAN" and insert instead --UNITED STATES PATENT OFFICE--; and that the said Letters Patent should be read with this correction therein.

Signed and sealed this 21st day of September, A. D. 1943.

(Seal)

Henry Van Arsdale,  
Acting Commissioner of Patents.